

## UNITED STATES PATENT OFFICE

2,669,534

## PRODUCTION OF ALLOYS

William Henry Richardson, Datchet, England,  
assignor to Langley Alloys Limited, Langley,  
England, a body corporate of Great Britain

No Drawing. Application February 19, 1951,  
Serial No. 311,808

Claims priority, application Great Britain  
February 20, 1950

8 Claims. (Cl. 148—11.5)

1

This invention relates to the production of alloys and more especially to aluminium bronzes consisting of copper and from 8-12% aluminium with optionally up to 8% of any one or more of the elements iron, nickel, cobalt and manganese, and in which bronzes smaller proportions of other elements such as antimony, arsenic, bismuth, chromium, lead, magnesium, phosphorus silicon or zinc each in amounts not exceeding 0.3% may be present intentionally or as impurities.

Normally, for highly stressed components, aluminium bronzes are employed in the wrought condition having been hot worked at temperatures of about 800-1050° C. depending on the aluminium content and the presence of additional constituents to the binary alloy, the working temperatures being higher in the case of those alloys containing smaller proportions of aluminium within the specified range, and also when the additional constituents, such as iron, nickel, cobalt, manganese and/or chromium are present and lower in the case of alloys containing higher percentages of aluminium within the specified range or when additional elements such as silicon, tin and/or zinc are present.

The invention has for its object to provide an improved method of manufacturing articles from alloys and especially from aluminium bronzes of the character in question by which consistently homogeneous products having improved mechanical properties and particularly high fatigue strength, may be readily and consistently obtained.

Further and favourable objects will appear from the following description.

Broadly stated, the improved method of manufacturing articles from aluminium bronzes according to the invention consists in subjecting the material to a heat treatment within the temperature range 800° C. up to about 1050° C. according to the particular constitution of the alloy, to bring it substantially to a beta condition where substantially the whole of the aluminium is in solid solution and then quenching the material to below 600° C. virtually to retain this condition and to ensure that any alpha particles that may be present are in the form of a fine dispersion, prior to reheating the alloy for its final hot working or forging to a finished shape within a temperature range at which alpha particles are still present.

Following the quenching treatment and prior to final hot working, the alloy may if desired, be further heat treated within the temperature range 400 to 800° C. and by this means the

2

quantity and distribution of alpha particles can be more closely controlled.

In this condition the alloy is reheated to the required temperature and subjected to its final hot working to the required shape.

Depending upon the particular constitution of the alloy and the method of final heating and working, a temperature range found suitable for such hot working is 700° C.-1000° C.

10 The alloy as cast may be subjected to hot rolling, forging or extrusion to produce bar stock prior to the treatment, or heat treatment and subsequent quenching according to the present invention may be effected immediately after the 15 aluminium bronze has been cast conveniently in chill moulds, or at any time after it has been subjected to the preliminary hot work and prior to the final working.

It will be appreciated that the pressed, forged, 20 rolled or extruded article may be finally subjected to a tempering or artificial ageing treatment at a temperature not above the temperature at which it has been hot worked and that in this after-treatment the article may be 25 quenched in a suitable medium or cooled slowly or allowed to cool naturally in air to the temperature of the ambient atmosphere.

In the practice of the invention, as applied to an aluminium bronze including 11% aluminium, 5% iron, 5% nickel and 1% manganese with the remainder copper, except for the impurities referred to hereafter, the billets are preliminarily hot worked by rolling, forging or extruding into suitable stock at about 900° C.

35 Thereafter they are subjected to heat treatment as described at 910° C. so that a substantially beta condition is produced and continue the treatment for a period of  $\frac{1}{4}$  of an hour following by quenching, and any alpha particles present are in the form of a fine dispersion uniformly distributed throughout the matrix. In this condition the stock is then ready for final forming to shape, preferably by being extruded, pressed into moulds or shaped dies or rolling or forging at 800-890° C., after which treatment the material possesses an extremely fine grain structure in which the alpha particles are uniformly distributed throughout the matrix and are of a size not exceeding 50 microns.

50 The shaped articles, such as turbine or compressor blades are then, if desired subjected to the final optional artificial tempering treatment at 600-700° C. when they are found to exhibit enhanced mechanical properties and especially high fatigue strength even at elevated tem-

## 3

peratures and under working conditions involving considerable vibration.

Although hitherto it has been possible to produce an aluminium bronze of this type possessing high proof stress and tensile strength, the methods heretofore employed for producing such properties have resulted in lack of uniformity, but by the improved method according to the present invention it is possible to produce a far superior combination of properties and further, these properties can be consistently obtained. Typical properties of the aluminium bronze treated as aforementioned are as follows:

0.1% proof stress \_\_\_\_\_ tons per sq. inch 45.1 15  
 Maximum stress \_\_\_\_\_ do 56.7  
 Elongation \_\_\_\_\_ percent 16  
 Endurance limit \_\_\_\_\_ tons per sq. inch +25

Analysis of a specimen of the aluminium bronze showed the following impurities to be present:

|            | Percent |
|------------|---------|
| Arsenic    | 0.005   |
| Chromium   | 0.001   |
| Lead       | 0.01    |
| Silicon    | 0.07    |
| Tin        | 0.005   |
| Zinc       | 0.01    |
| Magnesium  | 0.05    |
| Phosphorus | 0.01    |

In another example of the practice of the invention as applied to an aluminium bronze having the following composition:

|            | Percent |
|------------|---------|
| Aluminium  | 10.72   |
| Iron       | 5.26    |
| Nickel     | 5.15    |
| Manganese  | 0.23    |
| Arsenic    | 0.005   |
| Chromium   | 0.001   |
| Lead       | 0.015   |
| Silicon    | 0.05    |
| Tin        | 0.007   |
| Zinc       | 0.02    |
| Magnesium  | 0.05    |
| Phosphorus | 0.01    |

with remainder copper, the treatment is carried out as in the first example except that after rolling at 900° C. and cutting to size, if necessary, the billets are heated at 930° C. for three quarters of an hour and then quenched in water before final shaping by hot work at 800° C.-900° C. and artificial tempering for 2 hours at 650° C.

Typical specimens showed the following properties:

0.1% proof stress \_\_\_\_\_ tons per sq. inch 38.5  
 Maximum stress \_\_\_\_\_ do 55.0 60  
 Elongation \_\_\_\_\_ percent 19

When subjected to alternating stresses as in the fatigue test, several specimens of this material withstood 25,000,000 reversals of stress when the stress applied was 26 tons per sq. inch before fracturing.

A specimen of material of similar composition and size when produced by conventional methods and when subjected to such alternating stresses withstood only 1,200,000 reversals of stress when the applied stress was 26 tons per sq. inch before fracture, while another specimen when subjected to a lower stress of only 25 tons per sq. inch fractured after 1,800,000 reversals.

Such known material exhibited the following mechanical properties:

0.1% proof stress \_\_\_\_\_ tons per sq. inch 34.25  
 Maximum stress \_\_\_\_\_ do 57.25  
 Elongation \_\_\_\_\_ percent 10.5

The invention is also particularly advantageous in the reheating of billets for hot working when a high frequency induction process of heating is used.

In normal extruded or rolled bar stock as used for forgings the alpha particles occur as comparatively large and often elongated laves. In heating for hot working, time must be allowed for these large particles of alpha to be taken into solution in the beta matrix and consequently when high frequency induction methods of heating are used it may not be possible to take the fullest advantage of the extremely rapid rate at which this method of heating raises the billets to the desired temperature since much of the alpha would remain still undissolved.

If however, the billets are treated in accordance with this invention the very fine distribution of alpha in the billets prior to re-heating enables the heating to be effected at a much more rapid rate while still obtaining the necessary degree of solution of the alpha particles in the beta phase and full advantage can therefore be taken of the rapid rate of heating and the consequent increase in production which is possible by high frequency heating.

By the present invention, forged aluminium bronzes of enhanced mechanical properties may be conveniently and consistently manufactured.

What I claim is:

1. A method of manufacturing articles from aluminium bronzes consisting of copper and from 40 8-12% aluminium with smaller proportions of other ingredients comprising subjecting the article to a heat treatment within the temperature range 800° C. up to about 1050° C. according to the particular constitution of the alloy, to bring it substantially to a beta condition where substantially the whole of the aluminium is in solid solution and then quenching the material to below 600° C. virtually to retain this condition and to ensure that any alpha particles that may be present are in the form of a fine dispersion, and then reheating the alloy and subjecting it to final hot working to a finished shape at a temperature within the range 800°-900° C. at which alpha particles are still present.

2. A method of manufacturing articles from aluminium bronzes according to the preceding claim wherein for controlling the quantity and distribution of the alpha particles in the alloy, it is subjected, after quenching and prior to final hot working, to a soaking treatment within the temperature range 400-800° C.

3. A method of manufacturing articles from aluminium bronzes according to the preceding claim 1 wherein the alloy as cast is subjected to preliminary hot work at 900° C.±10° C. to produce stock which is then subjected to the heat treatment at a higher temperature followed by quenching to condition the material for the final hot working to shape by forging.

4. A method of manufacturing articles from aluminium bronzes according to the preceding claim 1 wherein the shaped article is finally subjected to a tempering or artificial ageing treatment at a temperature not above the temperature at which it has been hot worked.

5. A method of manufacturing articles from aluminium bronzes according to the preceding claim 1 and consisting of 11% aluminium, 5% iron, 5% nickel and 1% manganese with remainder copper except for impurity elements wherein the cast alloy is subjected to preliminary hot work at about 900° C. followed by heat treatment at 910° C. for about three quarters of an hour, uniformly to disperse the alpha particles throughout the matrix prior to final hot working to shape at 800-890° C.

6. A method of manufacturing articles from aluminium bronzes according to the preceding claim 5 wherein the heat treated alloy is quenched prior to storage for subsequent hot working, and the shaped article is subjected to a final artificial tempering treatment at 600-700° C.

7. A method of manufacturing articles from aluminium bronzes according to the preceding claim 1 and consisting of 10.72% aluminium 5.26% iron, 5.15% nickel and 0.23% manganese with remainder copper except for impurity elements, wherein the cast alloy is subjected to

10

preliminary hot work at about 900° C. followed by heat treatment at 930° C. for about three quarters of an hour, uniformly to disperse the alpha particles throughout the matrix prior to final hot working to shape at 800-900° C.

8. A method of manufacturing articles from aluminium bronzes according to the preceding claim 1 wherein the heating for final hot working to shape is effected by high frequency induction.

WILLIAM HENRY RICHARDSON.

References Cited in the file of this patent

UNITED STATES PATENTS

| Number    | Name  | Date          |
|-----------|-------|---------------|
| 2,075,509 | Davis | Mar. 30, 1937 |

OTHER REFERENCES

"Aluminum Bronze," by "Copper Development Association," London (Reprint 1939), page 42.  
 "Metallurgia," March 1950, pages 242, 243.